

## 1

2,854,458

## COMPLEX HEAVY METAL SALTS

Walter Reppe, Ludwigshafen (Rhine), Herbert Friederich, Worms, and Hans Laufenschlager, Ludwigshafen (Rhine), Germany, assignors to Badische Anilin- & Soda-Fabrik Aktiengesellschaft, Ludwigshafen (Rhine), Germany

No Drawing. Application July 14, 1955  
Serial No. 522,183

Claims priority, application Germany July 15, 1954

14 Claims. (Cl. 260—326.5)

This invention relates to complex heavy metal salts and to a method of manufacturing such salts. More particularly, the invention concerns complex salts of iron, cobalt, nickel or copper with carboxylic acid amides.

An important object of this invention is to provide new complex compounds of heavy metals and a method of producing these complex compounds.

Another object is to provide complex compounds by the interaction of iron, cobalt, nickel or copper salts with a substituted carboxylic acid amide bearing at least one organic substituent on the nitrogen atom of the amido group.

Other objects will be apparent from the more detailed description of the invention.

These objects are accomplished according to this invention by reacting a salt, preferably a halogenide of iron, cobalt, nickel or copper, with a substituted carboxylic acid amide.

The carboxylic acid amide should contain at least one organic substituent, preferably a hydrocarbon radical, on the nitrogen atom of the amido group. Suitable carboxylic acid amides derive from primary and secondary aliphatic, cycloaliphatic, heterocyclic and aromatic amines and from aliphatic, cycloaliphatic, aromatic or heterocyclic carboxylic acids. Such carboxylic acid amides are, for instance, dimethylformamide, N-methylacetamide, N-ethylbenzoic acid amide, propionic acid pyrrolidide and N-methylacetanilide. Other suitable carboxylic acid amides are the lactams of aminocarboxylic acids and their N-alkyl derivatives, such as pyrrolidone-2, N-methylpyrrolidone-2, caprolactam, dimethylacetamide, dimethylbenzamide, N-formylhexamethylene imine, N-formylpyrrolidine, di-n-dodecylpropionamide, dimethyl-palmitinamide, distearylacetamide, cyclohexane carboxylic acid dimethylamide and N-cyclohexylacetamide. The amides chiefly used are dimethylformamide, dimethylacetamide, pyrrolidone and N-methylpyrrolidone. The length of the chain of the carboxylic acids and the amines shall be from 1 to 20 C-atoms, as for example with distearylacetamide or dimethylpalmitin amide. All of the aliphatic, cycloaliphatic and heterocyclic compounds used should be saturated. As heavy metal salts the bromides and iodides of iron, cobalt, nickel and copper are preferably used. Acetates, propionates or acrylates of nickel or cobalt may also be used.

The complex compounds are easily formed by mixing the initial materials and slightly heating this mixture, preferably to a temperature between 40° C. and 160° C. The reaction may be carried out in the presence of a solvent, such as tetrahydrofuran, methanol, ethanol or butanol, or while an excess of the carboxylic acid amide is used. A deep green or a blue solution or melt is soon formed thereby, from which the complex compounds separate in crystalline form when the solution or the melt is cooled. In some cases it is advantageous to add the metal salts to the acid amides in the form of

## 2

aqueous solutions and to distill off the water afterwards in vacuo or azeotropically. If an excess of the carboxylic acid amide is used and the complex compound formed is soluble in the carboxylic acid amide, it is possible to separate the complex compound by the addition of liquids having a poor dissolving power for the complex compounds, for instance, by the addition of ethers, esters or hydrocarbons. The complex compounds may also be separated and/or purified by extracting the melt or the solution and/or by recrystallization. As a rule, for 1 mole of the metal salt from 3 to 10 moles of the carboxylic acid amide are used.

5 The new complex compounds are usually crystalline, stable compounds having a definite melting point. They contain as a rule for one molecule of the metal salt from 3 to 8 molecules of the carboxylic acid amide.

10 The new complex compounds may be characterized by the following general formula



15 In this formula Me is iron, cobalt, nickel or copper, these metals having an atomic number from 26 to 29; Hal is a halogen, x is an integer from 2 to 3, corresponding to the valence of the metal Me, y is an integer from 3 to 8 and A is a carboxylic acid amide containing at 20 the nitrogen atom of the amido group at least one organic substituent which is preferably a hydrocarbon radical. The term "hydrocarbon radical" includes alkyl radicals, such as methyl, ethyl, propyl or butyl, as well as alkylene radicals occurring in lactams between the amido and the 25 oxo group.

30 Complex compounds containing water of crystallization separate occasionally from solutions containing water. Most of them can, however, be converted into water-free complex compounds by recrystallization from water-free solvents, such as water-free tetrahydrofuran.

35 The complex compounds are, as a rule, soluble in water and in several organic solvents, such as alcohols, acetone, chloroform and tetrahydrofuran. The solutions of these compounds are usually stable, but sometimes when they are heated the complex compounds decompose and the simple metal salt precipitates. If the complex compounds are heated under reduced pressure to a temperature above their melting point, they often 40 decompose and the carboxylic acid amide distills off while the metal salts remain behind.

45 While the new complex compounds are easily soluble in different solvents, they may be used with advantage to carry out chemical reactions such as carbonylations where the difficultly soluble simple metal salts do not give a satisfactory result. The complex acid amides of nickel bromide have an excellent catalyzing action in the synthesis of acrylic acid or the derivatives thereof at raised temperature and increased pressure. The complex cobalt halides are efficient catalysts in the carbonylation of methanol into acetic acid or the carbonylation of amines, especially tertiary amines, into amides under similar conditions. In these cases, the presence of organic solvents is prohibitive of the use of the simple heavy metal salts. Moreover the catalytic activity of the complex compounds are far superior to that of the simple salts.

50 The invention is further illustrated but not limited by the following examples in which the quantities are given in parts by weight unless otherwise indicated.

Example I

55 20 parts of nickel-II-bromide are dissolved in 40 parts of N-methyl pyrrolidone-2 while stirring and slowly heating the mixture to a temperature of 150° C. After the nickel bromide has completely dissolved, the solution is cooled, and 20 parts of a crystalline dark blue complex

compound separate. The crystal sludge is separated from the mother liquor and the latter is covered with a layer of 80 parts of diethyl ether. Within 24 hours, 18 additional parts of the same complex compound separate. After recrystallization from tetrahydrofuran, the complex compound has a melting point of 105° C. It contains for one molecule of nickel-II-bromide three molecules of N-methyl pyrrolidone-2.

*Example II*

15 parts of nickel bromide are dissolved in 50 parts of dimethylformamide while the mixture is heated to 100° C. During cooling, 14 parts of a crystalline blue complex compound  $\text{NiBr}_2 \cdot 3\text{HCON}(\text{CH}_3)_2$  separate. After the addition of 50 parts of ether to the mother liquor, 14 additional parts of the complex compound are obtained. The complex compound has a melting point between 123° C. and 126° C. after washing with ether and drying under vacuum.

*Example III*

2 parts of nickel bromide are dissolved in 90 parts of pyrrolidone-2 at a temperature of 120° C. The hot solution has a bluish-green color which changes when the solution is cooled to room temperature, to dark green. During cooling, 7.5 parts of a green complex salt  $\text{NiBr}_2 \cdot 8$  (pyrrolidone-2) crystallizes. The complex salt is washed with ether and dried under vacuum. It melts at 125° C. When heated in tetrahydrofuran, the complex compound loses part of the pyrrolidone and converts into a blue compound  $\text{NiBr}_2 \cdot 3$  (pyrrolidone-2) which is insoluble in tetrahydrofuran in the cold and has a melting point of 155° C.

*Example IV*

32.6 parts of cobalt bromide hexahydrate are dissolved while heating to 125° C. in 80 parts of pyrrolidone-2. From this solution, 52 parts of a reddish-violet complex compound  $\text{CoBr}_2 \cdot 3$  (pyrrolidone-2) (melting point 125° C.) crystallizes after the solution has been cooled and kept for 24 hours. By the addition of ether to the mother liquor, 30 additional parts of the same complex compound can be isolated.

*Example V*

A solution of 10 parts ferric chloride in 100 parts of dimethylformamide is evaporated at room temperature under a reduced pressure of 0.6 millimeter Hg to dryness. 18 parts of a yellowish-brown crystalline mass are obtained which yields after having been digested three times with water-free ether and after having been dried in vacuum, 15 parts of a yellowish crystalline complex compound having a melting point of 68° C. to 70° C. This complex compound, having the composition  $\text{FeCl}_3 \cdot 3$ -dimethylformamide is insoluble in ether, petroleum ether and ethyl acetate and dissolves in water, alcohols, tetrahydrofuran, and acetone.

*Example VI*

A solution of 10 parts of cupric bromide in 100 parts of dimethylformamide is evaporated at room temperature under a reduced pressure of 0.6 millimeter Hg to dryness. 18 parts of a black crystalline mass are obtained which is twice digested with 80 parts of water-free ether and dried under vacuum, whereby brilliant black crystals of a complex compound of the composition  $\text{CuBr}_2 \cdot 4$ -dimethylformamide and having a melting point of 76° C. to 78° C. are obtained. They dissolve easily in water, alcohols, tetrahydrofuran or pyridine. The complex compound is difficultly soluble in benzene and insoluble in ether, petroleum ether and ethyl acetate.

*Example VII*

20 parts of nickel chloride hexahydrate are dissolved in 50 parts of N-methyl pyrrolidone-2 while heated to 75° C. From the dark blue solution, 28 parts of a dark green complex compound separate when it is cooled. The crystals are filtered off, washed with N-methyl pyrrolidone-2, absolute ether and dried under vacuum. The complex compound which has the composition  $\text{NiCl}_2 \cdot 3\text{N-methylpyrrolidone-2}$  melts at 79° C. to 80° C.

150° C. From the dark blue solution, 28 parts of a dark green complex compound separate when it is cooled. The crystals are filtered off, washed with N-methyl pyrrolidone-2, absolute ether and dried under vacuum. The complex compound which has the composition  $\text{NiCl}_2 \cdot 3\text{N-methylpyrrolidone-2}$  melts at 79° C. to 80° C.

*Example VIII*

10 parts of nickel iodide are dissolved while heating to 100° C. in 100 parts of dimethylformamide. The obtained brown solution is filtered and evaporated under a reduced pressure of 0.5 millimeter Hg at room temperature (about 25° C.) to dryness. 16.5 parts of a brownish-green residue remain behind. By washing this residue with tetrahydrofuran, green crystals of a complex compound of the composition  $\text{NiI}_2 \cdot 5$ -dimethylformamide are obtained which melt after drying under vacuum at 88° C. to 90° C.

20

*Example IX*

11.3 parts of caprolactam are dissolved in 30 parts of tetrahydrofuran. To this solution 3.6 parts of finely pulverized nickel bromide are added and the mixture is then boiled for 5 hours under reflux. After cooling 12.0 parts of a yellow residuum are separated. By recrystallizing this from a large quantity of tetrahydrofuran pale yellow crystals are obtained which melt at 121° C. and correspond to the formula  $\text{NiBr}_2 \cdot 4$  caprolactam.

30

*Example X*

15 parts of nickel bromide are dissolved in 50 parts of dimethylacetamide while heating. By combining the dark blue solution with 100 parts of dry ether 31 parts of a blue-green crystalline precipitate are obtained. After washing the precipitate with dry ether and drying it in vacuo it melts at 82° C. Its constitution corresponds to the formula  $\text{NiBr}_2 \cdot 3$  dimethylacetamide.

40

*Example XI*

To a melt of 100 parts of N-methylacetanilide 21.8 parts of nickel bromide are added at 120° C. while stirring and the mixture is cooled down after an hour. The dark green crystal mass is triturated three times with 200 parts of dry ether. The bottoms left are 55 parts of a blue-green compound having the formula  $\text{NiBr}_2 \cdot 3\text{N-methylacetanilide}$  and melting at 128° C.

The invention is hereby claimed as follows:

1. A complex heavy metal salt of the general formula



wherein Me is a metal with an atomic number from 26 to 29, Hal is a halogen, x is an integer from 2 to 3, y is an integer from 3 to 8 and A is a carboxylic acid amide of the formula  $\text{R}-\text{CO}-\text{NR}_1\text{R}_2$ , wherein R constitutes a radical selected from the group consisting of hydrogen, alkyl, cycloalkyl, aryl hydrocarbon, and radicals which together with  $\text{R}_2$  constitute a bivalent alkylene radical,  $\text{R}_1$  constitutes a radical selected from the group consisting of hydrogen, alkyl, cycloalkyl, aryl hydrocarbon, and radicals which together with  $\text{R}_2$  constitute a bivalent alkylene radical, and  $\text{R}_2$  constitutes a radical selected from the group consisting of alkyl, cycloalkyl, aryl hydrocarbon, radicals which together with R constitute a bivalent alkylene radical, and radicals which together with  $\text{R}_1$  constitute a bivalent alkylene radical.

2. A complex heavy metal salt of the formula



3. A complex heavy metal salt of the formula



4. A complex heavy metal salt of the formula



5. A complex heavy metal salt of the formula



6. A process of manufacturing a complex heavy metal salt which comprises reacting one mol of a halide of a metal having an atomic number from 26 to 29 with 3 to 8 mols of a carboxylic acid amide of the formula  $\text{R}-\text{CO}-\text{NR}_1\text{R}_2$ , wherein R constitutes a radical selected from the group consisting of hydrogen, alkyl, cycloalkyl, aryl hydrocarbon, and radicals which together with  $\text{R}_2$  constitute a bivalent alkylene radical,  $\text{R}_1$  constitutes a radical selected from the group consisting of hydrogen, alkyl, cycloalkyl, aryl hydrocarbon, and radicals which together with  $\text{R}_2$  constitute a bivalent alkylene radical, and  $\text{R}_2$  constitutes a radical selected from the group consisting of alkyl, cycloalkyl, aryl hydrocarbon, radicals which together with R constitute a bivalent alkylene radical, and radicals which together with  $\text{R}_1$  constitute a bivalent alkylene radical.

7. A complex heavy metal compound comprising one molecule of a halide salt of a metal having an atomic number from 26-29, inclusive, in complex combination with 3-8 molecules of dimethylformamide.

8. A complex heavy metal compound comprising one molecule of a halide salt of a metal having an atomic

number from 26-29, inclusive, in complex combination with 3-8 molecules of pyrrolidone-2.

9. A complex heavy metal compound comprising one molecule of a halide salt of a metal having an atomic number from 26-29, inclusive, in complex combination with 3-8 molecules of N-methylpyrrolidone-2.

10. A complex heavy metal salt of the formula



11. A complex heavy metal salt of the formula



12. A complex heavy metal salt of the formula



13. A complex heavy metal salt of the formula



14. A complex heavy metal salt of the formula



References Cited in the file of this patent

UNITED STATES PATENTS

2,581,905 Carr \_\_\_\_\_ Jan. 8, 1952

OTHER REFERENCES

Pfeiffer: Organische Molekülverbindungen, Stuttgart, Verlag von Ferdinand Fenke (1927), (Zweite Auflage), pp. 112-5.

Andre: Beilstein (Handbuch, 4th ed.), vol. 2, page 178 (1920).